

July 27, 1943.

M. G. WHITFIELD

2,325,156

METHOD OF COATING WIRE

Filed Dec. 11, 1939



## UNITED STATES PATENT OFFICE

2,325,156

## METHOD OF COATING WIRE

Marshall G. Whitfield, Louisville, Ky., assignor  
to Reynolds Metals Company, New York, N. Y.,  
a corporation of Delaware

Application December 11, 1939, Serial No. 308,693

8 Claims. (Cl. 117—114)

This invention relates to the coating of wire, and more particularly to the coating of a metal wire with metals of the general character represented by aluminum. While applicable to the coating of wires of other metals with other coating metals, the invention has been found of particular utility in the coating of ferric wire with aluminum.

In the coating of ferric wire with aluminum or the like as heretofore practiced, the aluminum coat is likely to have succeeding portions along its length which are of different thicknesses, and this is particularly true if a relatively thick coating of aluminum is desired. Inasmuch as the utility of the coating is ordinarily limited by its least thickness, the regions of increased thickness merely add to the weight and cost without any corresponding increase in benefit, while the irregular cross section resulting is itself a disadvantage.

The cause for these variations in thickness is not precisely known, but without wishing to be limited to the correctness of the following theory, it is now believed that these variations in thickness are attributable to the presence of a relatively tenacious oxide film at the surface of the molten bath. Such film is apparently drawn onto the emerging wire along with the coating metal, and tends to adhere to the latter as it congeals on the wire. While the tenacity and elasticity of such surface film permits temporary adhesion to the coating, the resistance to the drag of this film across the molten metal, together with its weight as it tends to follow the wire out of the bath, causes a more or less periodic rupture of the film. Thus not only are portions of the film left on the emerging coated wire, to vary its thickness and other characteristics, but the ruptured film, sliding down the emerging metal, owing to the elastic action of the film following each rupture, tends to wipe some of the coating from the emerging wire, thereby accentuating the variations in thickness.

Whatever the cause of the variations in coating thickness heretofore obtained, I have discovered that coatings of substantially uniform thickness can be obtained, and this thickness may be made several times greater than that heretofore obtained, if the wire is actuated so as to cause it to move rapidly and transversely with respect to the surface of the bath where it is emerging therefrom, through an orbital path that may take a variety of forms but for convenience is preferably made a closed circular path.

It is therefore an object of the present invention to provide a method for coating wire whereby a substantially uniform coating of controlled thickness may be obtained.

5 Another object of this invention is to provide a method of the type characterized whereby a coating of materially greater thickness may be obtained than has heretofore been the case.

10 Another object of this invention is to provide a method of the type characterized which is particularly applicable to the coating of ferric wire with aluminum and which enables a substantially uniform and predetermined coating to be formed on the wire that may be several times the thickness heretofore obtainable.

15 Other object will appear as the description of the invention proceeds.

The method of the present invention is capable of being carried out in a variety of ways 20 and with a wide variety of apparatus, one of which is diagrammatically illustrated on the accompanying drawing, but it is to be expressly understood that the drawing is for purposes of illustration only, and is not to be construed as a definition of the limits of the invention, reference being had to the appended claims for that purpose.

25 The drawing illustrates schematically apparatus that may be used for effecting the desired movement of the emerging wire.

30 In accordance with the present invention the wire, where it emerges from the bath, is made to move rapidly, and transversely to the surface of the bath, through a predetermined orbital path 35 which, within the broader aspects of the present invention, may take a variety of forms as will be apparent to those skilled in the art from the present disclosure, but for convenience of operation and simplicity of apparatus required it is desirably a path that is circular in form.

35 Referring to the apparatus illustrated in the drawing, 10 designates any suitable container for the bath of molten coating metal, heated in any suitable way to maintain the same properly fluid. The wire 11 to be coated is introduced into said bath 10 in any suitable way, as by means of a nozzle 12 which opens beneath the surface of the bath. From the nozzle 12 the wire 11 passes around any suitable roller 13 mounted in any suitable way as by means of a bracket 14. 40 From the roller 13 the wire 11 emerges from the bath, preferably at right angles to the surface thereof, and as here shown the wire then passes 45 through a cooling pipe 15 of any suitable length,

form and character (and constituting no part of the present invention).

Then the wire passes through a constraining ring 16, preferably mounted in a ball bearing 17 supported in any suitable way as by an annular frame 18. As here illustrated the ball bearing 17 is retained in the frame 18 by a hinged ring 19 pivoted to the frame 18 at 20 and provided with a pivoted locking bolt 21 and nut 22 for co-operation with a slot 23 in said frame 18. Thereby, after backing off the nut 22, the bolt 21 may be pivoted around its axis 24 to release the locking member 19, whereupon the latter may be swung about its pivot 20 to gain access to the bearing 17 for inspection or renewal.

From the constraining ring 16 the wire passes upwardly through means for moving the wire through its designed path. Where, as here, said path is circular in form said mechanism may take the form of a pulley 25 suitably mounted in a frame 26 as by having its hub 27 which cooperates with bearing member 28 retained against displacement from said bearing by means of a locking ring 29 suitably secured to said hub as by screw 30. Eccentrically mounted in the pulley 25 is a member surrounding wire 11 for impressing on the wire its circular movement. As here shown an annular plug 31, preferably made of a relatively soft metal, such as aluminum, so as not to scratch the surface of the coating, is suitably mounted on the pulley, preferably for ready attachment and detachment, as by means of the ball bearing 32 in an annular block 33 secured in the pulley 25. The unit composed of the plug 31 and its bearing 32 may be conveniently attached to the block 33 by a plurality of screws 35, and said block 33 may be secured in the recess 34 by a plurality of screws 36. Pulley 25 is driven in any suitable way from a motor or other source of power not shown.

From the plug 31 the wire passes upwardly over a roller 37 and thence to any suitable drum or wire take up machine.

Pulley 25 is preferably rotated at a speed on the order of 1200 R. P. M. While considerable variation in the speed of rotation of pulley 25 may be made, experience has seemed to demonstrate that a rotation on the order of 1000 R. P. M. is a critical minimum speed for apparatus of the type illustrated, the effects obtained by the practice of the present invention disappearing, largely if not entirely, if the rotative speed is reduced below this R. P. M.

The rotation of pulley 25 with its plug 31 causes the wire to move through a cylindrical path whose limits are diagrammatically indicated by the solid and dotted lines of the wire 11 in the drawing. The upper and lower limits of the movement of the wire are of course determined by the rollers 13 and 37, but other suitable means may be employed if desired. The constraining ring 16 keeps the wire in a nearly cylindrical path and prevents the wire from bellying out toward a loop so as to develop undue stresses therein.

Where the wire 11 emerges from the free surface 38 of the bath, the wire is rapidly traversing a circular path of small diameter, while the inertia of the molten metal causes it to pile up in the form of a wave at the advancing side of the wire, so that the effect of the movement of the wire through the metal extends an appreciable distance on either side of said path. Hence the rapid traverse of its path by the wire sets up a

circular area which by observation may be seen to be substantially free of oxide film, the movement of the wire apparently preventing the formation of a film within an area which is slightly larger than that embraced by the path of the wire. Accordingly the wire emerges through a surface that is substantially free of oxide film, so that the coating is not varied in thickness by portions of film adhering thereto or tending to wipe portions of the coating off the emerging wire, while the wave piled up in front of the rapidly moving wire apparently assists in effecting a thicker coating.

But whatever may be the physical explanation of the results obtained, experience has demonstrated that for wires of more than 0.10 inch in diameter, whereas the maximum average coating heretofore obtained was approximately 0.64 mil per side, thicknesses averaging from 1.75 mils to 2.0 mils per side may be regularly obtained by the practice of the present invention. With wires less than 0.10 inch in diameter the coatings obtained are somewhat less, but on the same order as compared with earlier accomplishments. The thickness of the coating obtained may be controlled to some extent by varying the speed of movement of the wire through the emerging surface of the bath.

Therefore, by the practice of the present invention, substantially uniform coatings, which are several times thicker than heretofore obtained, have been regularly secured by the practice of the present invention in the coating of ferric wire with aluminum. But while the invention is of particular utility in coating ferric wire with aluminum, it is not limited thereto but has utility where the presence of a film at the surface of the coating bath may cause irregularities in the thickness of the coating.

While the present invention has been described in connection with an apparatus which causes the wire to traverse a closed path in the form of a circle, it will now be apparent to those skilled in the art that such a path is not of the essence of the invention, although for simplicity of apparatus that character of path has obvious advantages. By varying the apparatus used, however, the wire may be caused to pass through closed paths of a variety of other forms, and it is also apparent that other apparatus may be designed for causing the wire to move through a circular path or other form of paths. Various other changes may be made in the details of the procedure without departing from the spirit of this invention, and therefore reference is to be had to the appended claims for a definition of the invention.

What is claimed is:

1. The method of providing a wire with a relatively thick and substantially uniform coating which includes the steps of passing the wire through a bath of molten coating metal and moving said wire transversely to its length where it emerges from the surface of said bath to cause the wire to rotate along a circular path of small diameter and at a rate in excess of 1000 R. P. M.

2. The method of coating ferric wire with aluminum to provide said wire with a relatively thick and substantially uniform aluminum coating which includes the steps of passing said wire through a bath of molten aluminum and moving said wire transversely to its length where it emerges from the surface of the bath to cause said wire to rotate along a circular path of small diameter and at a rate in excess of 1000 R. P. M.

3. The method of providing a wire with a relatively thick and substantially uniform coating which includes the steps of passing the wire through a bath of molten coating metal, and establishing an uninterrupted wave in engagement with the wire where it emerges from the surface of the bath by continuously moving said wire at a relatively high speed in the same direction through a closed orbital path traced at the surface of the bath.

4. The method of providing a wire with a relatively thick and substantially uniform coating which includes the steps of passing the wire through a bath of molten coating metal and continuously moving the emerging wire cylindrically in the same direction and at a relatively high speed to trace a closed orbital path on the surface of the bath.

5. The method of providing a wire with a relatively thick and substantially uniform coating which includes the steps of passing the wire through a bath of molten coating metal and continuously moving the emerging wire in the same direction and at a relatively high speed to trace a closed orbital path at the surface of the bath whose dimensions approximate the maximum movement of the wire transversely of its length.

6. The method of coating ferric wire with aluminum to provide said wire with a relatively

thick and substantially uniform aluminum coating which includes the steps of passing said wire through a bath of molten aluminum and continuously moving said wire at a relatively high speed around the periphery of a small area at the surface of said bath to generate an uninterrupted wave in contact with the emerging wire.

7. The method of coating ferric wire with aluminum to provide said wire with a relatively thick and substantially uniform coating which includes the steps of passing said wire through a bath of molten aluminum and continuously moving said wire at a relatively high speed and in the same direction through a closed orbital path which is substantially cylindrical in form.

8. The method of coating ferric wire with aluminum to provide said wire with a relatively thick and substantially uniform coating which includes the steps of passing said wire through a bath of molten aluminum and continuously moving said wire at a relatively high speed and in the same direction through a closed orbital path, the magnitude of movement of said wire at the surface of the bath approximating the maximum magnitude of movement of said wire transversely of its length.

MARSHALL G. WHITFIELD.